

## UNITED STATES PATENT OFFICE.

GEORGE F. SHEEHAN AND HUGH A. GILLEN, OF SEATTLE, WASHINGTON.

## FUEL BRIQUETTE.

No Drawing.

Application filed September 24, 1921. Serial No. 502,994.

*To all whom it may concern:*

Be it known that we, GEORGE F. SHEEHAN and HUGH A. GILLEN, citizens of the United States, residing at Seattle, in the county of 5 King and State of Washington, have invented a certain new and useful Improvement in Fuel Briquettes, of which the following is a specification.

The present invention contemplates the 10 utilization of low or inferior grades of coal, such as lignite or sub-bituminous coals, and to compound therewith, binding, coking or carbonizing combustible substances to produce fuel briquettes of a relatively high degree of efficiency.

With this end in view the invention consists in compounding the lignite or sub-bituminous coal with the desired percentage of binding material or binder, such as tar pitch, 20 asphalt, or gilsonite and the desired percentage of a coking or carbonizing substance, such as free burning sulphur, all of which are thoroughly pulverized and mixed, and molding the resultant compound into 25 briquettes of the desired shape and size.

In carrying out the invention our composition consists of pulverized coal; a binder, such as pulverized tar pitch, asphalt or gilsonite; a coking agent, such as pulverized 30 sulphur; a clinker eliminator, such as pulverized sea shells; a smoke and soot minimizer, such as pulverized zinc; and a substance to prevent the disintegration of the briquette during the burning of the same, 35 such as pulverized manganese.

In preparing the composition we prefer to use the elements or ingredients in approximately the following proportions—viz: 90 per cent of pulverized coal; 7 per cent of 40 pulverized coal tar pitch, asphalt or gilsonite; one and one half per cent of pulverized sulphur; a half of one per cent of pulverized sea shells; a half of one per cent of pulverized zinc; and a half of one per cent of pulverized metallic manganese.

In some cases depending upon the grade of coal to be briquetted, the sea shells, zinc and manganese may be omitted, or any one of the same when desired, in which event 50 additional pulverized coal is added to replace the element or elements omitted.

The elements or ingredients in the above mentioned proportions are next placed in a mixer of any well known form, which mixer 55 is maintained in a heated condition during

the mixing operation at an approximate temperature of 325 degrees Fahrenheit.

When the elements or ingredients comprising the composition have been properly mixed, the resultant mixture is then fed 60 through suitable conduits to a briquette forming press of any well known form, wherein said mixture is compressed under the desired pressure to produce briquettes of the selected size, shape and density. The 65 said briquettes on being discharged from said press are then ready for shipment.

However, if coke is desired and required the resultant product or briquettes discharged from the press are then placed in a 70 coking oven and baked at a suitable temperature to produce a high grade coke of high commercial value.

In briquetting the substances hereinbefore enumerated, using only a binder, it was 75 found in repeated tests that the briquettes thus formed, because of the rapid evolution of the gases during the period of combustion, disintegrated rapidly when the melting point of the binder was reached, while, briquettes embodying a percentage of sulphur, in addition to a suitable binder were caused to coke or carbonize rapidly during the period of combustion, thus preventing disintegration of the same, the reason for such coking or carbonizing action taking place, being that during the initial stages of combustion the sulphur is rendered viscous and plastic, but as the heat or temperature increases 80 during the later stages of combustion the viscosity of the sulphur diminishes and the tendency for the sulphur to pass into a crystalline form or state increases, thus causing coking or carbonization of the briquettes. 85

It will thus be apparent that by adding 90 a predetermined percentage of sulphur to the substance to be briquetted, which sulphur must not be confused with the organic or non-combustible sulphur inherent in some grades of lignite and sub-bituminous coals, that such addition of sulphur will change the lignite or sub-bituminous coals during the combustion period to a coked or carbonized state. In other words, the properties, effect and usefulness of the substances 100 enumerated are changed by the interaction and addition of the sulphur and the identity of the said substances substantially destroyed. 105

Another advantage obtained by the above 110

described coking or carbonizing action is the substantial retention in the unconsumed portion of the treated fuel during the period of combustion of the volatile matter inherent in the substances aforementioned.

By thus retarding the expulsion of the volatile matter the B. t. u. ratio of the treated fuel is considerably increased over that of the aforesaid substances in a raw or natural state.

Repeated analysis of both the raw and treated substances indicated the following satisfactory results: an increase of from 1500 to 3000 B. t. u.'s; a substantial increase of the fixed carbon ratio and a similar increase of the volatile matter ratio in the treated substances over that of the raw substances.

Sulphur, when treated with a bituminous binder about the melting point of sulphur, produces a vulcanized binder.

What we claim is:

1. A fuel briquette containing lignite and a bituminous binder vulcanized by sulphur, said binder being composed of approximately 4 parts bitumen and 1 part of sulphur.

2. A fuel briquette containing approximately ninety per cent of lignite, and the remainder containing a bituminous binder vulcanized with a relatively small quantity of sulphur.

3. A fuel briquette composed principally of lignite and having a bituminous binder and containing a relatively small quantity of added sulphur, adapted to vulcanize the binder and produce coking of the fuel.

In witness whereof, we hereunto subscribe our names this 19th day of September A. D. 1921.

GEORGE F. SHEEHAN.  
HUGH A. GILLEN.